

Dec. 3, 1940.

W. A. DARRAH

2,223,603

## EQUIPMENT FOR HEAT TREATING

Original Filed July 15, 1938

4 Sheets-Sheet 1



Fig. 1.

## *Inventor*

William A. Darral.

Dec. 3, 1940.

W. A. DARRAH

2,223,603

EQUIPMENT FOR HEAT TREATING

Original Filed July 15, 1938 4 Sheets-Sheet 2



Fig. 2.

Inventor  
William A. Darrah

Dec. 3, 1940.

W. A. DARRAH

2,223,603

EQUIPMENT FOR HEAT TREATING

Original Filed July 15, 1938

4 Sheets-Sheet 3



Inventor

William A. Darrah

Dec. 3, 1940.

W. A. DARRAH

2,223,603

EQUIPMENT FOR HEAT TREATING

Original Filed July 15, 1938 4 Sheets-Sheet 4



Fig. 6.



Fig. 5.

Inventor

William A. Darrah

## UNITED STATES PATENT OFFICE

2,223,603

## EQUIPMENT FOR HEAT TREATING

William A. Darrah, Chicago, Ill.

Original application July 15, 1938, Serial No. 219,332. Divided and this application November 10, 1938, Serial No. 239,860

6 Claims. (Cl. 266—4)

This application is a division of application Serial No. 219,332 filed July 15, 1938, and issued Dec. 26, 1939, as Patent No. 2,184,972.

This invention relates to apparatus used for 5 treating metals and particularly the ferrous metals including steels of various types. One important application of the apparatus which forms the subject of invention is in connection with the so-called carburizing of steel or various 10 materials which consists in forming a case of highly carburized steel on the outer surface of an article.

This apparatus may be utilized to form other 15 compounds or gases on a metallic base as for example a nitride case and a mixture of carbide and nitride cases. Other compounds such as volatile metals as for example zinc may be added to the surface of the metal being treated utilizing some phases of my invention.

20 In order to simplify the disclosure I will confine the description of the apparatus largely to the specific operation of carburizing steel articles, although it should be understood that my invention is by no means confined to this field only.

One of the objects of my apparatus is to form 25 a strong hard resistant surface on a steel article. Another object of my invention is to form a surface on steel articles economically and rapidly.

30 Another object of my invention is to provide equipment which will utilize natural gas, city gas or the so-called liquid fuel gases such as butane and propane for carburizing operations without the production of excessive soot or coke 35 on the metal being treated.

Another object of my invention is to provide means whereby various relatively "rich" carbon bearing gases may be utilized for carburizing.

40 Another object of my invention is to provide simple, automatic and economical means for completely carburizing and heat treating steel articles the operations including carburizing, reconditioning grain size, quenching, drawing, washing, etc., so that the steel article when it leaves is completely treated.

Other objects of my invention will be apparent 45 from the drawings, description and claims appended hereto.

50 Referring to the drawings Figure 1 shows a typical plan view of one form of my invention.

Figure 2 shows a side elevation of the carburizing zone of this furnace partly broken away to indicate the interior construction. Figure 2 55 is a partial section taken along the line II—II as

indicated in Figure 1 and as further indicated in Figure 3.

Figure 3 shows a typical cross section through the furnace portion of my invention taken along line III—III of Figure 2.

Figure 4 shows a side elevation partially broken away indicating quenching devices, discharge door and other details of my invention.

Figure 5 shows a side elevation partially broken away indicating a general arrangement of a draw 10 oven. Figure 6 indicates a typical tray or fixture loaded with material to be treated.

Referring to the drawings 1 indicates a carburizing furnace provided with loading vestibule 2 and loading table 3.

15 4 indicates a cooling zone attached to the discharge end of the carburizing furnace and 5 indicates a reheating furnace arranged to reheat the material preparatory to quenching after the material has been cooled in zone 4 or otherwise. 20

6 indicates a quenching housing or vestibule connected to spray washing station 7 and spray rinse zone 8 adjacent thereto. A recirculating draw oven 9 is shown located at the end of the rinsing zone 8.

25 Similar numbers refer to similar parts on the various drawings and figures.

The loading platform 3 consists preferably of a structural steel frame work although obviously any suitable material may be employed.

30 A series of fixtures or trays 10 are loaded while resting on platform 3 and then pushed either manually or by the means of operating cylinder 11 into vestibule 2 in the position shown in dotted lines and indicated by numeral 12.

35 At the proper time of the cycle, either controlled by the operator or automatically by an electric timer, operating pushing cylinder 13 pushes tray 12 into carburizing chamber 1 through operating door 14. The electric timer 40 may be any of the conventional types now available on the market. Of course loading vestibule 2 is closed by manually operating door 15 to prevent leakage of air in or gases out during the cycle. This vestibule is also supplied with purging gases, such as a mixture of products of complete combustion through pipe 16, from gas generator 16A, which also supplies gas to the cooling chamber and quench vestibule.

45 The carburizing furnace itself may be constructed in a variety of ways but I prefer the general type of construction shown herewith in which heat is supplied by a series of radiant members such as tubes 17 which may be located either above or below the work to be heated and 55

which are provided with a burner 18, burner block 19 and exhaust flue 20 which leads to a duct 21 located beneath the furnace or at some other convenient point. Radiant member 17 naturally expands and contracts with changes of temperature and, therefore, is provided with a flexible seal or joint 22 which is filled with sand or other granular material. This construction provides for flexibility without permitting gases to leak into or out of the furnace chamber. The object of the construction is to provide a leak proof arrangement such that products of combustion or air within the combustion chamber cannot enter into the furnace chamber and conversely the atmosphere within the furnace chamber cannot enter into the combustion chamber. Since if all joints were bolted metal to metal there would be very substantial expansion which would cause cracking or breaking. The construction indicated provides a certain amount of flexibility by permitting the radiant tube member 17 to move in the cup member 22 by displacing the granular material. Referring to Figure 3 it will be noted that the radiant tube member 17 is sealed to the furnace shell 1 in an air tight manner to prevent leakage. Radiant member 17 it will be noted extends transversely across the heating chamber and curves downwardly dipping into the sand filled seal of member 22.

Member 22 extends downwardly as indicated and is tightly attached to the bottom plate of the furnace.

Since sealed member 22 is attached to the bottom plate of the furnace and radiant member 17 is attached to the vertical side walls of the furnace and both are sealed to their respective plates it will be evident that we have a continuous metal contact except for the expandable joint within the sand seal.

The housing or carburizing furnace which may to advantage be constructed of steel plate properly reinforced as indicated is made so that all joints are tight. The housing should then be insulated with heat resisting insulation as indicated by the layers 24 and the filling material 25 above the arch of the furnace.

The interior of the furnace should be constructed of refractory capable of withstanding high temperatures continuously in the presence of a strongly reducing atmosphere as this is ordinarily used to obtain the carburizing results desired. I have found that a porous refractory is of decided advantage for this service providing the outer face is well plastered with a refractory cement. All refractory material within the heating zone of the furnace should preferably be extremely low in iron oxide and similar compounds which may be readily reduced by temperatures ranging from 1600 to 1800° F., in the presence of hydrogen, carbon monoxide or other strongly reducing gases such as methane, and ethane. I have designated this layer of refractory material by the numeral 26.

It is to be noted that the refractory material subjected to strongly carburizing atmospheres is subject to failure not from melting as the temperatures used ordinarily range from 1600 to 1800° F. The refractory material is subject to failure by the reduction of iron oxide or similarly readily reducible compounds under the influence of various reducing gases as was cited above. The action of the reducing gases is at least two-fold. In the first place by converting iron oxide to metallic iron the bond which holds the refractory together is broken allowing the refractory

to crumble away. This results partly from a change in volume of iron as against iron oxide and partly because of the different nature of the material.

Of course if iron oxide is reduced by such gases as methane and ethane, as mentioned above, free carbon in the form of soot is always deposited in the pores of the refractory. These conditions can be eliminated for practical purposes by using the type of refractory specified above. Other effects of course are likely to be obtained when refractories containing compounds readily reducible by the reducing gases mentioned above are made.

A series of cross piers 27 are provided at intervals transversely across the furnace and between the radiating members. These piers should be made of strong materials and are used to support rails 28, 29 and 30, etc., on which the trays or other fixtures carrying the materials to be treated slide. The whole furnace is supported on a foundation indicated by 31.

At the discharge end of furnace chamber 1, a pusher 32 is located, arranged when actuated, to push the tray out of carburizing furnace 1 into cooling zone 4. In this zone the loaded trays are allowed to cool to temperatures ranging from 700 to 1200° or even over wider limits depending on the critical limits of the steel being treated. This chamber is tightly housed and consists substantially of a tight box or container hermetically sealed at one end to the carburizing furnace 1, and at the other end to the reheat furnace 5. Rails 33 are provided in this zone similar to those provided on loading table 3, so that as the trays 35 are pushed out of chamber 1 they will slide on rails 33 until opposite pusher 34 and in the position shown in dotted by numeral 35. As the trays reach this point cylinder 34 is actuated pushing the trays out of cooling zone 4 through doorway 36 into reheating furnace 5, where the temperature is raised preferably to around 1400° or higher to pass the critical temperature of the steel. When the tray reaches the end of reheat furnace 5 and assumes the position shown by the dotted tray 37, cylinder 38 pushes the tray into quenching chamber 6 as described below. Quenching chamber 6 is provided with an elevator member 39 raised and lowered by cylinder 40. In the bottom portion of chamber 6 quench liquid such as oil or, if desired, water is maintained. Cylinder 40 lowers elevator 39 into the quench liquid 41 thus quickly cooling the metal and producing the desired metallurgical characteristics.

The cylinders such as 32, 34, 38, and 42 may be operated sequentially by means of conventional interlocks (not shown) as is well known.

After a proper hesitation beneath the liquid to permit cooling of the steel to the desired temperature cylinder 40 lifts the elevator and tray to the operating level at which time pusher 42 is actuated and the tray is pushed into the washing zone 7. This washing zone consists of a series of sprays 76A supplied with washing liquid which is usually water with cleaning compounds dissolved therein. A pump 43 rotated by a motor 44 delivers the liquid to the spray nozzles at high pressures and large volumes as required. This type of equipment is well known.

The trays are pushed successively the length of one tray passing gradually through the washing zone and the rinsing zone, allowing ample time to remove oil, grease, carbon, dirt, coke and other foreign materials.

The rinsing zone is provided with a motor 45 and pump 46 which serves to supply clean water for removing all traces of washing compound. If this is not done the compound is likely to dry 5 on the steel parts causing an unsightly appearance. I prefer to use washing liquids strongly heated preferably close to 200° F. This, however, is an operating detail which may be varied to suit working conditions.

10 After leaving the rinsing zone the trays are pushed successively and intermittently through a draw oven as indicated in Figure 5.

In this oven the material is reheated gradually and uniformly to temperatures ranging from 300 15 to 700 or 800° depending again on the nature of the steel and the results to be obtained. It should be understood that wherever temperatures are specified they are given with a view of obtaining great toughness and hardness of the 20 outer layer of carburized steel and toughness and strength in the inner layer of steel. Other results may be obtained by this invention and are not to be excluded. Other results may require different operating temperatures and times.

25 The draw oven 9 shown in Figure 5, is supplied with circulating hot gases from duct 50 indicated in Figure 1. Duct 50 is arranged to receive the products of combustion from both the carburizing furnace 1 and the reheat furnace 5. These 30 products of combustion pass from the radiant combustion chambers 17 through the flexible joint 22 into down-comer 20 and finally connect to longitudinal flues 21 which run the entire length of the furnaces. Duct 51 connects with 35 the longitudinal duct beneath the carburizing furnace and duct 52 connects with the duct beneath the reheat furnace. Obviously these ducts may be put above the floor or beside the furnace if it is found more convenient to do so. Duct 51 40 is provided with a draft control damper 53 and duct 52 has a similar draft control damper 54. The two ducts connect to riser 55 which in turn leads the combined products of circulating combustion into duct 50 and then into the intake of fan 56 which delivers the hot gases into draw oven 9 at a point 57 located beneath the rails 58 45 on which the trays 59 are carried. Since the trays are of open or latticed construction the hot gases passing into the oven in space 57 travel upward, around and through the interstices of the trays and leave by means of spaces 60 between plate 61 which form the upper portion of the draw oven. The circulating gases thus enter plenum chamber 62 from which they pass to duct 55 53 which leads them back again to the recirculating fan. A control damper 64 in duct 50 may be operated by a thermostatically controlled motor in any conventional manner and thus draws more or less products of combustion into the circulating fan to maintain the temperature of the 60 circulating gases constant.

A thermostatic device 65 such as a sensitive couple placed in the circulating air stream in passage 57 serves to open or close damper 64 as required.

65 It will be evident that the hot circulating gases which utilize waste heat from the furnaces serve to give a closely controlled draw to the steel parts which have been carburized, cooled, reheated and quenched.

This oven also serves as a drying oven to remove the water from the washing and rinsing process and may be so used exclusively, if it is not desired to draw and temper in the steel pot. 70 In most cases the drawing operation serves to

toughen and soften the inner core of steel thus increasing the strength and durability of the product. Since the carbon content of the carburized shell on the outer surface of the steel is higher than the carbon content of the core, temperatures which will draw the core satisfactorily will not soften the shell appreciably.

75 After the trays have been pushed successively through the draw oven occupying in turn each of the positions indicated they finally come to the positions shown as 66 in Figure 5, after which they are pulled or pushed into vestibule 67. Vestibule 67 serves as a seal or hood to prevent excessive leakage in or out of draw oven 9. Succeeding position 68 provides a place for the trays 10 to cool before unloading and reloading.

15 It will be apparent that the trays have thus made the complete cycle of the apparatus having been submitted consecutively to each of the operations. Since the timing may be controlled by 20 an automatic timer or electric clock all times in carburizing, cooling, reheating and drawing may be accurately controlled. Furthermore, since temperatures and atmospheres are closely controlled the entire process gives a uniform product 25 having predetermined characteristics.

20 Referring to Figure 6, tray 70 may be taken as a typical unit used in my process but I do not wish to be restricted to this particular design as any commercial trays properly suited for this 30 process may be employed.

25 The tray 70 consists of a frame 71 which is sufficiently rugged to permit satisfactory pushing of the entire load. The frame 71 surrounds a lattice indicated by 72 formed from a number of 35 transverse and longitudinal bars. Preferably the entire tray is cast in one single integral piece, but if desired it may be formed in several sections dove-tailed or otherwise fastened together.

30 At the junction of the bars forming the lattice or at other points as required, a series of hub or supporting members indicated by 73 are provided. Any one of these members may be formed on the tray to suit the loading conditions required. A series of fixtures 74 may be provided 40 to slip into the hollow portion of hubs similar to 73 and these fixtures 74 support gears or other parts indicated by 75. It is understood that the trays will be loaded as desired and a typical installation may represent a load of 800 or 1000 45 pounds of steel to each tray which may weigh, by way of example, 200 to 300 pounds. Naturally these ratios and arrangements will vary widely with the nature, size and type of articles being treated and the kind of treatment given.

50 It will be apparent that in the apparatus here described products of combustion are excluded from the chamber in which the steel articles are heated so that it is possible to absolutely control the nature of the atmosphere in contact with the steel being treated. This is an essential feature of this invention in that proper control of the chemical and physical condition of the atmosphere is essential for obtaining the results 55 desired.

55 I am aware that carburizing has been performed by heating steel articles in a closed chamber in contact with carburizing gases. This process, however, has not met all requirements for numerous reasons among which are slowness of forming a desired case, difficulty in controlling the type and depth of case and the presence of large amounts of soot or coke on the surface of the steel.

70 75 Various expedients have been proposed to over-

come some of these difficulties but from my practical experience in this field I find that these expedients are not satisfactory.

In my invention I introduce carburizing gases into my furnace both above and below the trays carrying the work, as for example, by means of upper inlets 16 and lower inlets 11. I provide a number of these inlets along the length of travel of the work preferably placing them every three or four feet apart for purposes of control. These inlets may be connected to a suitable source of carburizing gas. I prefer to use either natural gas, propane or city gas direct without dilution or addition when it is desired to produce a carbon case on the surface of the work. In the past such a procedure would coat the surface of the steel heavily with soot or coke. This coating has several obvious objections. In the first place, it is difficult to remove and requires costly and expensive handling or polishing to entirely remove it as it is strongly adherent. If it is not fully removed it naturally causes serious wear in the devices utilizing the gears or other equipment treated.

25 A further objection to the soot is the fact that it apparently delays and retards the penetration of carbon into the steel.

In my apparatus I have found that while I provide a number of inlets for the natural gas both above and below the work, it is preferable to introduce the gas principally at the discharge end of the carburizing furnace at a point where the articles are about to leave the treatment. The carburizing gas will flow backward toward the loading end and promptly fill the entire chamber with atmosphere.

If gas is introduced the full length of the chamber sooting is likely to occur in the early stages with consequent slowing up of the carburizing reaction or a reduction of the percentage of carbon in the case.

Carbon of course first collects in the outer layer of steel and gradually penetrates to the interior of the steel. The concentration of carbon is naturally higher in the outer layers initially and lower in the inner layers. Most articles require for maximum hardness and durability a layer of hyper eutectoid in the outer layer, just below this a strata of eutectoid and below this 50 a final layer of hypo-eutectoid. If soot deposits occur they may retard the addition of carbon to the outer layer but of course they do not retard the diffusion of carbon from the outer layer into the interior of the steel. Soot deposits, therefore, 55 may be objectionable by causing a lower percentage of carbon in the case distributed over the entire band.

By my apparatus the carburizing gas, as for example natural gas, may be partly above the material being treated and partly below. The gas as added eventually comes in contact with the highly heated radiant chambers made of alloy or other heat resisting material. These chambers may range from 1800 to 2000° or over and 60 serve to crack the methane and other hydrocarbons in the gas. The degree of cracking depends on the time of contact, the temperature of which the gas is heated and the velocity of circulation of the atmosphere within the carburizing chamber. Naturally, having an intensely hot zone in the lower portion of the furnace violently circulating atmosphere streams are produced, and the atmosphere within the carburizing chamber is 65 kept well mixed and in rapid motion.

70 75 The breaking down of methane and other hy-

drocarbons naturally deposits some free carbon around the combustion chamber and the adjacent refractory walls and produces large amounts of hydrogen. The hydrogen serves as a dilutant for the incoming new quantities of methane in the natural gas and therefore protects it against rapid decomposition by the well known laws of mass action.

As a result of this condition it is only necessary to provide a proper ratio of hydrogen and inert gases to the amount of methane and hydrocarbon gases so that the deposit of carbon on the steel is reduced to a rate approximately equal to that at which it will be absorbed by the steel.

Further the hot cracked gases appear to be in a nascent or active condition and a greatly accelerated rate of carburization of the steel results.

It should be understood that while I have described my apparatus as applied to steel it may also be used with tungsten, chromium and other metals.

It should be understood that the statements made in this specification relating to reasons for obtaining the specially advantageous results which are secured, represent my theory as to operating principles and are not necessarily actual facts.

It is apparent that there is a rapid and violent circulation throughout the zone of the furnace occupied by the steel being carburized. It is also evident that the temperature of the gases doing the carburizing is higher than the temperature of the steel since the gases pass over the intensely hot radiating chambers at the bottom of the furnace and travel upward around the work being carburized. These two points I believe are of great importance in reducing the time required for carburizing and increasing the depth of case and the amount of carbon absorbed.

These factors also make it possible to carburize with less additional atmosphere than is required in the case of present day muffle type furnaces in which the carburizing chamber is of necessity maintained at a relatively uniform temperature at the top and bottom of the chamber. The present carburizing chambers or muffles being made of alloy and, therefore, very costly are kept as small as possible. It is necessary to keep the present carburizing furnaces small in order to reduce the expansion and warping which is an extremely serious item in the case of a large muffle. In the case of the furnace which I have invented there is no large muffle but merely a brick wall which is ordinarily formed of insulating refractory plastered with a refractory cement to seal the pores against the entrance of the carburizing gas. As a result of my construction many of the limitations of the present furnaces are removed and I can build a furnace of my design in any desired size in any dimension, using commercial materials now available. This is not practical with present day carburizing muffles, owing to the limitations of making and maintaining large alloy boxes or containers which of course must be kept air tight.

In the case of equipment of my design, making a longer furnace merely means building the steel container of greater length and lining it with firebrick as shown. More of the small individual radiating units are then added as required. Obviously the same principle applies to increasing the width of my furnace.

By introducing the new carburizing atmosphere which may be methane, propane, butane or various other hydrocarbon gases or a mixture of these,

or hydrocarbon containing CO, nitrogen, etc., at the upper portion of my heating zone, I obtain one set of conditions and I obtain a different set of conditions by introducing the carburizing gases 5 in the lower portion of the heating zone. By controlling the amount introduced above and below the work to be carburized I have a type of control of the nature of the case formed on the steel, which is not possible in present day carburizing units.

10 I prefer to exhaust a small amount of the gases at each end of the carburizing furnace partly to provide space for introducing new gas and partly to provide a visual indication of the nature of the 15 gas within the furnace. By lighting the stream of gas which leaves the furnace at the ends, I am able to produce a flame which has distinctive characteristics depending on the composition of the gas. Thus an extremely rich gas will burn 20 with a deep red or reddish yellow flame, producing considerable smoke, while a leaner gas will produce a lighter colored flame and a gas of hydrogen and CO will produce a flame which is still more transparent. It has been the experience of 25 operators using my equipment that as long as the nature of the flame is held constant the gas condition within the furnace is substantially constant and the nature of the case produced on the steel is substantially constant.

30 Another point which I have found of great advantage in the furnace which I have invented is the fact that the necessary temperatures for producing a given degree of case, other things being equal, are considerably less in my 35 furnace than in the case of the older type of muffle.

I attribute this fact partly to the rapid circulation of the gases due to the thermal difference caused by an intensely hot radiating member in 40 the bottom of the furnace and partly to the fact that the gases passing over the steel or other material being treated are hotter than the steel itself.

45 It will be understood that my invention includes a process of carburizing and also the equipment for accomplishing this result. My invention includes also a cycle and process as well as the associated equipment, in which the waste heat from the high temperature operation 50 is utilized in the low temperature operation.

My invention also includes various other features as set forth in the specifications and the attached claims.

55 It will be understood I do not wish to be restricted to any special set of temperature, time or gas conditions as these are ordinarily varied to suit the requirements of the material being treated. I have found, however, that my process and equipment permits substantially shortening the time, lowering the temperature and increasing the depth and carbon content of the case. The relative degree to which these different advantages exist are subject to control 60 depending on conditions to be obtained.

65 By adding ammonia to the atmosphere which I use for obtaining the carburized case I am able to add a substantial amount of nitrogen to the case which forms on the steel. In this manner I am able to produce a case which contains both 70 nitride and carbide and thus has many of the characteristics ordinarily associated with the treatment of steel in a molten bath of sodium cyanide.

75 As indicated above, I may use as atmosphere straight natural gas without adding any from of

diluting material. Under these conditions the cracking of the gas liberates hydrogen, a portion of the carbon being absorbed by the steel and a portion of the carbon being precipitated as coke or graphite, some on the walls of the furnace 5 and some on the heat radiating member or other parts. The presence of this accumulation of carbon appears to ultimately retard the cracking of the methane in the natural gas thus preserving more of the gas for use in forming the carburizing case on the steel. This is my theory as to one of the reasons why I am able to carburize a given quantity of steel to a given depth with much less carburizing gas than is ordinarily used in present day conventional furnaces.

10 15 It will be apparent, therefore, that the atmosphere within my furnace will ordinarily contain a considerable amount of free hydrogen which has proved to be of no objection in the case of any commercial application so far tested.

20 In the opening of the doors for loading and discharging of my furnace there is naturally a slight leakage of gas outward from the doors and of air into the furnace chamber. This has proved to cause no difficulty but accounts for the 25 presence of a small amount of nitrogen and oxides of carbon within the furnace chamber. Of course vestibules are provided as indicated to reduce this condition to a minimum but my experience has been that quite substantial amounts 30 of air may enter the furnace chamber without causing difficulties.

Water vapor may be present in a small degree but it is desirable to exclude water vapor as far 35 as possible when a high carbon content is desired on the surface of the steel.

40 I wish to emphasize that in the equipment which I have invented I maintain an intensely hot source of radiation in the lower portion of the carburizing chamber while the material being carburized or otherwise treated is located in another portion of the chamber, usually the upper portion. As a result of this condition, the atmosphere within the carburizing chamber comes in contact with intensely hot surfaces, 45 acquires a portion of this intense heat and then travel upward by thermal circulation, coming in contact with the cooler steel or other articles being carburized. As a result of this condition, the hydrocarbon gases are hotter than the steel 50 which is being carburized, even when the steel is up to its maximum temperature. This condition causes the soot, which is precipitated on the steel in other competitive processes now in use, to deposit in those portions of the furnace which 55 are hot rather than on the steel. This condition leaves the steel relatively clean and free from deposits of coke and soot, which are characteristic of other methods of carburizing now in use. The deposit of coke or soot on the surface of the steel is a serious disadvantage from many standpoints. It retards the rate of carburization because it forms a coating or shield and keeps the carburizing gases from having intimate contact with the steel. Naturally a heavy 60 coating of soot or coke requires a cleaning and in the case of present commercial process this cleaning is quite difficult and costly.

65 It will be noted that in present commercial apparatus an alloy muffle forms the containing 70 chamber in which the steel being treated is enclosed, together with the carburizing gas. It is necessary to heat the muffle throughout its cross section to a fairly uniform temperature to avoid excessive warping, cracking and deteriora- 75

tion. This condition means that the rapid thermal circulation is missing and the temperature of the muffle is substantially the temperature of the steel being treated. Therefore, present commercial processes lack the substantial difference in temperature between the steel being carburized and the gas containing the carburizing material. It appears that the desired results can only be obtained in the best measure by utilizing the thermal circulation which this process and type of construction provides. Forced circulation by fans does not give the results obtainable by this process, possibly because the difference in temperature between the circulating gases and the material being carburized is not as great as in the case of the thermal circulation which I utilize.

It is notable that articles treated by my process come out clean and free from coke and contain no visible soot. While I am familiar with many of the present day carburizing processes I have found none which give this condition. It should be noted that this condition is obtained without the addition of foreign gases of any kind and no oxidizing agents or oxidizing gases are essential to my process although they may be present to a limited degree without interfering with the operation of my process.

A substantial portion of my invention, therefore, is the means of obtaining clean and uniformly carburized articles in a minimum time and with a lower temperature than is customary today.

Owing to the rapid thermal circulation of the hot carburizing gases and the fact that they are at a higher temperature than the metal being carburized, carbon is added with great uniformity which is not the case with muffle furnaces now in use.

40 By the term "material support" used in the claims I intend to bring out the structure which supports the material being treated within the furnace. It is obvious that the supports must extend to the floor or foundation by some intermediate means and it is intended that the heating means be below the material being carburized and not necessarily below the entire portion of any support.

I claim:

50 1. A metal treating apparatus of the type described consisting of a carburizing chamber, a cooling chamber attached thereto, a reheat chamber attached to said cooling chamber, a quench chamber attached to said reheat chamber, a washer attached to said quenching chamber and a draw oven attached to said washer, and a mechanism for moving material to be treated through said chambers, the whole forming an integral unit for successively and continuously treating materials.

2. A metal treating apparatus of the type described consisting of a refractory carburizing chamber, a metallic vestibule sealed thereto in a tight manner, closure means for said vestibule to prevent entrance of air into said chamber during loading, a quench chamber sealed to said

carburizing chamber to prevent entrance of outside air, a washer attached to said quenching chamber, and a draw oven attached to said washer and a mechanism for moving the material to be treated through said chambers, the whole forming an integral unit for successively and continuously treating metals.

3. An apparatus for carburizing metals which consists of a refractory carburizing chamber resistant to disintegration by carburizing atmosphere, support means for the material to be treated in said chamber, a combustion chamber located within said carburizing chamber below said material being treated, sealed from communication with said carburizing chamber to prevent products of combustion from entering said carburizing chamber, an inlet for carburizing gas into said carburizing chamber located adjacent the end of said carburizing chamber and near said radiant chamber, arranged to lead the carburizing gas toward said combustion chamber so that carburizing gas on entering is heated to a conditioning temperature by said combustion chamber.

4. An apparatus for carburizing metals including a carburizing chamber formed with walls of refractory, a support for material being carburized, a radiant heating member located below said material on said support, and an inlet for carburizing gas adjacent said heating member arranged to lead the carburizing gas into contact with said radiant member so that said heating member may preheat said carburizing gas after passing through said inlet.

5. An apparatus for carburizing metals consisting of a carburizing chamber with refractory walls, a support for material being carburized, a radiant heating member in the lower portion of said chamber, said radiant chamber extending transversely across said carburizing chamber and being provided with a sand seal near the point at which said radiant member leaves said carburizing chamber, and an inlet for carburizing gas adjacent said heating member, said inlet located and arranged to lead said carburizing gas into contact with said radiant heating member after passing through said inlet.

6. An apparatus for carburizing metals consisting of a carburizing chamber with refractory walls, a support for the material being carburized, a series of tubular combustion chambers arranged below the material being carburized and arranged transversely across said carburizing chamber, a separate burner arranged to deliver combustible materials into the interior of each combustion chamber, each combustion chamber being sealed to prevent entrance of air into said carburizing chamber, and gas tight means connecting each of said combustion chambers with an exhaust duct arranged to carry products of combustion from said apparatus, and an inlet for carburizing gas adjacent one of said combustion chambers and located and arranged to lead said carburizing gas into contact with said combustion chamber.

WILLIAM A. DARRAH.